

# United States Patent Office

3,832,132  
Patented Aug. 27, 1974

1

3,832,132

## PROCESS FOR IMPROVING THE DIMENSIONAL STABILITY OF WOOL-CONTAINING FABRICS

Giuliana C. Tesoro, Dobbs Ferry, N.Y., and Stephen B. Sello, Cedar Grove, and Rudolf F. Wurster, Weehawken, N.J., assignors to J. P. Stevens & Co., Inc., New York, N.Y.

No Drawing. Filed Nov. 8, 1968, Ser. No. 774,499  
Int. Cl. D06m 13/38

U.S. Cl. 8—127.6

7 Claims

### ABSTRACT OF THE DISCLOSURE

This invention concerns a novel process for modifying proteinaceous substrates comprising treating said substrates with polyfunctional reagents derived from urea and heating the treated substrate until the desired modification takes place.

The present invention relates to novel processes for treatment of proteinaceous materials and more particularly processes for enhancing the properties and characteristics of textiles containing wool fibers and improved products obtained thereby.

Various methods have been devised for the treatment of textile fabrics containing wool in order to improve certain properties thereof. Particularly important to the wool industry are methods and compositions to bring about improvements in the dimensional stability and the felting characteristics of textiles containing wool fibers. Although many methods have been developed for wool treatment, relatively few give satisfactory results from the standpoint of improvement in dimensional stability and felting. Moreover, prior known methods frequently may deleteriously and adversely affect the appearance, handle, strength and other properties of the woolen textiles.

Accordingly, it is the object of the present invention to provide novel processes for imparting improved properties to proteinaceous materials, particularly wool-containing textile materials, which overcome the shortcomings and disadvantages associated with prior methods and compositions.

It is a further object of the present invention to provide novel processes for imparting excellent properties and characteristics to wool-containing textiles which avoid the drawbacks of prior methods and compositions.

It is a further object of the present invention to provide novel processes for imparting to wool-containing textile material excellent properties of dimensional stability and resistance to felting.

It is a further object of the present invention to provide woolen textiles having improved properties, particularly dimensional stability.

It is a further object of the present invention to provide processes for treating wool-containing textile materials without adversely affecting the appearance, handle, strength and other desirable properties of the textile.

It is a further object of the present invention to provide processes for treating wool-containing fabrics which have desirable surface appearance after laundering, particularly minimal fuzziness.

In attaining the above objects, one feature of the present invention resides in imparting excellent properties and characteristics to proteinaceous materials by treating textile materials containing wool fibers with a selected group of polyfunctional compounds of a specified structure whereby the improvements in dimensional stability and other physical properties are achieved without adversely affecting the appearance, hand, strength and other desirable properties of the textile.

More particularly, a proteinaceous textile substrate such as wool and its blends is treated with a solution of poly-

2

functional composition represented by the structural formula:



wherein

A is selected from the group consisting of epoxyalkoxy, particularly wherein the alkoxy moiety has from 3 to 6 carbon atoms, Az, —NH—C<sub>a</sub>H<sub>2a</sub>Az, and —O—C<sub>a</sub>H<sub>2a</sub>Az, where a is an integer from 1 to 4, and m is an integer from 2 to 3, Az is



where R<sup>1</sup>, R<sup>2</sup>, and R<sup>3</sup> are independently selected from the group consisting of H and alkyl having from 1 to 4 carbon atoms,

R is selected from the group consisting of H and alkyl having 1 to 5 carbon atoms,

J is a divalent or trivalent organic radical, and

Q is selected from the group consisting of divalent aromatic and alkyl-substituted aromatic groups having 6 to 18 carbon atoms,

to deposit an amount sufficient to obtain the enhancement of properties sought, dried and cured at elevated temperatures until the properties of the substrate are enhanced.

While all of the above polyfunctional compositions function effectively as modifiers and enhancers of proteinaceous substrates, as in any large group, some members of the group, for various reasons, function more effectively than the others and for this reason are preferred. Thus, in the instant case, a more restricted group of compositions included within the above broad group, comprise the preferred compositions of this invention. These compositions are included within the structural formula:

(I)



wherein

A is selected from the group consisting of epoxypropoxy, Az, —NH—C<sub>a</sub>H<sub>2a</sub>Az, and —O—C<sub>a</sub>H<sub>2a</sub>Az, where a is a number from 1 to 4, m is a number from 2 to 3, Az is



where R<sup>1</sup> and R<sup>2</sup> are independently selected from the group consisting of H and alkyl having from 1 to 4 carbon atoms;

R is H or alkyl having 1 to 5 carbon atoms;

J is a divalent aliphatic or alicyclic radical, and

Q is methylphenylene.

In the preferred process embodiment, a woolen or wool blend substrate is contacted with an amount of one or more of the preferred treating agents, in the form of a liquid solution, sufficient to deposit a modifying or enhancing amount of agent and cured until the desired

enhancement of properties is obtained. Ordinarily the concentration of treating agent required varies between about 0.25 to 10% by weight with the true upper limit determined primarily by economics. The mode of application is not critical; padding, spraying, dipping or the like being applicable. Depending upon the initial concentration of agent utilized, the pickup varies between about 50% to about 300%. Normally the treated substrate is dried and cured at about 100° C. to 200° C. for about 3 to 6 minutes, longer times being acceptable.

A further feature of the present invention resides in treating wool-containing textile materials with a group of polyaziridinyl compounds and with selected co-reactants in order to further enhance and improve the dimensional stability and other physical properties of the textile without adversely affecting the appearance, hand, strength and other desirable properties thereof.

A more specific feature of the present invention resides in treating wool-containing textile materials according to a process hereinafter defined with a certain group of relatively high molecular weight polyaziridinyl compounds in the presence of selected polybasic acids of polyamino compounds whereby excellent properties are imparted to the textile.

The above, as well as other objects, features and advantages of the present invention will become apparent from the following detailed description thereof.

According to the present invention, novel processes are provided whereby wool-containing textile materials, particularly woven and knitted fabrics containing wool fibers, are treated with selected polyfunctional compounds to impart dimensional stability and other desirable properties to the textile product without substantially adversely affecting the appearance, handle, strength and other mechanical properties thereof.

It has been observed that the dimensional properties of wool-containing textile materials are considerably enhanced as a result of the novel processes of the present invention and further that the desired properties are obtained without causing undesirable discoloration, harshening or other undesirable side effects. Moreover, in accordance with a further aspect of the present invention, novel processes are provided whereby an enhancement in the physical properties of wool-containing textile materials, particularly dimensional stability, are obtained when the above-defined aziridine compounds are used in conjunction with co-reactants to be defined hereinafter which bring about an even greater improvement than was heretofore possible.

A detailed description of the substituents included within the formulae defining the polyfunctional compounds of this invention follows:

The compounds that are preferred for the present invention are polyfunctional compounds defined by Formula (I), *supra*.

Aziridinyl and oxiranyl compounds as defined by the symbol A in the various formulas which are suitable for purposes of the present invention may be obtained by several methods described in the chemical and patent literature. Briefly described, the class of compounds defined by Formula (I), *supra*, may be prepared by reacting an organic polyisocyanate with, preferably, an organic compound containing at least two amino groups to produce an intermediate having at least two isocyanate groups. Then the intermediate compound is reacted with a hydroxy-terminated 1,2-alkylenimine or hydroxy-terminated oxirane to obtain the desired product. It has been determined that compounds falling within the scope of the Formula (I), *supra* are exceptionally suitable for the treatment of wool-containing textile materials. It will be apparent from a consideration of the compounds encompassed by the present invention that the average molecular weight of the preferred compounds will range from about 1000 to about 6000. Such compounds are

commercially available or can be prepared by known methods from commercially available raw materials.

The following descriptive matter illustrates specific aspects of the various moieties that are used to produce the polyfunctional compounds of this invention.

#### GROUPS REPRESENTATIVE OF Q

| Name:                                                          | Composition                                                                       |
|----------------------------------------------------------------|-----------------------------------------------------------------------------------|
| Phenylene (o, m, or p)                                         | —C <sub>6</sub> H <sub>4</sub> —                                                  |
| Methylphenylene (various isomers such as 4-methyl-m-phenylene) | —C <sub>6</sub> H <sub>3</sub> (—CH <sub>3</sub> )—                               |
| (o, m, or p)-Phenylenedimethylene                              | —H <sub>2</sub> CC <sub>6</sub> H <sub>4</sub> CH <sub>2</sub> —                  |
| Biphenylene                                                    | —C <sub>6</sub> H <sub>4</sub> C <sub>6</sub> H <sub>4</sub> —                    |
| Methylenedi-(o, m, or p)-phenylene                             | —C <sub>6</sub> H <sub>4</sub> CH <sub>2</sub> C <sub>6</sub> H <sub>4</sub> —    |
| Benzylphenylene                                                | —C <sub>6</sub> H <sub>3</sub> (—CH <sub>2</sub> C <sub>6</sub> H <sub>5</sub> )— |
| Naphthylene                                                    | —C <sub>10</sub> H <sub>6</sub> —                                                 |

The residue J can be (a) divalent, or (b) trivalent.

(a) Illustrative of the residue J in the form of a divalent radical are the following:

- (II) (—CH<sub>2</sub>—)<sub>x</sub>, where x is a number from 1 to 100.  
 (III) (—C<sub>a</sub>H<sub>2a</sub>O—)<sub>x</sub>C<sub>a</sub>H<sub>2a</sub>, where a is a number from 1 to 4, and x is a number from about 1 to about 100, preferably from about 5 to about 40.  
 (IV) (—CH<sub>2</sub>CH=CHCH<sub>2</sub>—)<sub>u</sub>, which is derived from polybutadiene, wherein the average degree of polymerization, u is between about 6 and about 100.

- (V) —C<sub>a</sub>H<sub>2a</sub>(—OC<sub>a</sub>H<sub>2a</sub>—)<sub>x</sub>O—L—O(—C<sub>a</sub>H<sub>2a</sub>O—)<sub>y</sub>C<sub>a</sub>H<sub>2a</sub>—,

where

a is 1 to 4;

x and y independently are 1 to 100; and

L is a divalent alicyclic radical of 10 to 20 carbon atoms, C<sub>2</sub> to C<sub>20</sub> alkylene, or C<sub>2</sub> to C<sub>20</sub> alkylene having the chain interrupted by 1 to 10



groups in which R is alkyl having 1 to 5 carbon atoms.

In all instances, J is connected directly to nitrogen atoms, that is, the general formula is



wherein the molecular weight of J ranges from about 14 to about 5,500, and A, R, and Q have the definitions ascribed to them above.

For instance, suitable divalent radicals of the type represented by Formula (V) are provided by condensation products of the alkoxylate type which can be formed from any of the following starting compounds HO—L—OH which are given by way of example by

- (A) ethoxylation with approximately 10 to 125 mole-parts of ethylene oxide,  
 (B) propoxylation with approximately 8 to 95 mole-parts of propylene oxide, or  
 (C) alkoxylation with a proportionate mole ratio of higher or mixed alkylene oxides.

When J represents a trivalent radical, glycerin or similar triols can be used as starting materials.

The starting materials which can be used when J represents a divalent radical are listed as follows:

## STARTING COMPOUNDS HO-L-OH PRIOR TO ALKOXYLATION

|                      |                                                                         |
|----------------------|-------------------------------------------------------------------------|
| Ethylene glycol      | HO-CH <sub>2</sub> CH <sub>2</sub> -OH                                  |
| Propylene glycol     | HO-CH(CH <sub>3</sub> )CH <sub>2</sub> -OH                              |
| Trimethylene glycol  | HO-CH <sub>2</sub> CH <sub>2</sub> CH <sub>2</sub> -OH                  |
| Decamethylene glycol | HO-(CH <sub>2</sub> ) <sub>10</sub> -OH                                 |
| Diethylene glycol    | HO-CH <sub>2</sub> CH <sub>2</sub> OCH <sub>2</sub> CH <sub>2</sub> -OH |
| 2-butene-1,4-diol    | HO-CH <sub>2</sub> CH=CHCH <sub>2</sub> OH                              |



Typical of the methods whereby the aziridinyl compounds may be made is the procedure shown in Example 1 and the subsequent reaction with the reaction aziridine.

Illustrative of the above compounds are:

Epoxyalkoxy compounds as defined by the symbol "A" in the various Roman numeral formulas including (I) which are suitable for the purposes of the present invention are illustrated by the formulas below and by the preferred preparation of Example 3.

25





In carrying out the present invention, the wool-containing textile material which may be in any suitable form such as fiber, yarn or fabric may be treated with the polyfunctional compounds defined by Formula (I), generally by impregnation with a solution thereof.

The solvent vehicle may be aqueous or non-aqueous. The treating mixture of solvent and polyfunctional compound may be in the form of a solution, suspension, emulsion or the like. The textile material may be sprayed, padded, immersed, dipped, brushed or similarly contacted with the polyfunctional compound, thereafter dried and cured. Exposure to elevated temperature may be used to insolubilize the polyfunctional compound. Alternatively, the textile, after being contacted with the polyfunctional compound, may be permitted to stand for a brief period so as to achieve insolubilization.

If desired, the treated wool-containing textile material may thereafter be washed to remove residual soluble chemicals which may interfere or adversely affect the properties of the final product. Excellent dimensional stability is imparted to woolen textiles treated in the aforementioned manner. When laundered by conventional procedures commonly used for cotton or hydrophobic fibers, the woolen textile materials treated in accordance with the present invention as well as garments made from such woolen textile materials do not exhibit noticeable felting, fuzzy appearance, shrinkage or other undesirable properties which would deleteriously affect the final quality of the garment.

The present invention constitutes a considerable advance over what has gone heretofore inasmuch as the treatment with the selected polyfunctional compounds does not deleteriously alter the color, hand or other aesthetic properties of the woolen textile and, moreover, does not substantially adversely impair the tensile strength, tear strength, abrasion resistance and other important properties of the textile material.

In accordance with a further preferred aspect of the present invention, textile materials containing wool are treated with the aziridine compounds represented by the Formula (I) *supra* in combination with the coreactants as defined hereinafter to achieve even greater enhancement of the dimensional stability and other desirable properties of the textile products. Suitable co-reactants are polybasic acids and polyamine compounds particularly saturated aliphatic dicarboxylic acids containing from 2 to 12 carbon atoms and polyalkylenepolyamines containing, for example, from 4 to 20 carbon atoms and 2 to 5 nitrogen atoms. Representative examples of acids include succinic acid, adipic acid, sebacic acid, citric acid, tartaric acid, polyacrylic acid, and the like. Examples of polyamines include diethylenetriamine, tetraethylenepentamine, hydroxyethylmethylenediamine, polyethylenimines of wide molecular weight range, 1,3-diaminopropane, 1,6-diaminohexane, and the like.

In general, it has been observed that the co-reactants will accelerate insolubilization of the polyfunctional compound in or on wool and will drive the polymerization reaction to completion in a shorter period of time. In ad-

dition, it has been observed that in certain respects the resulting properties of the textile are superior to that treated with the polyfunctional compound alone. It is, however, to be noted that the invention does not require the presence of co-reactants in order to achieve satisfactory dimensional stability or other desirable properties in the wool-containing textile.

The treating mixture containing the polyfunctional compounds as defined by the structural Formula (I) and a vehicle therefor may take the form of a solution in organic solvents or water when feasible. The compounds may also be applied from aqueous emulsion which can be rapidly prepared by suitable choice of solvents and emulsifying agents. Because of their stability at room temperature over relatively long periods of time, solutions and emulsions of the treating agents of the present invention may normally be stored without special precautions being necessary.

According to a further more detailed aspect of the present invention, the wool-containing textile material may be treated with the above-defined polyfunctional compounds, either before or after dyeing because the treatment with aziridines does not alter or deleteriously affect the dyeing properties of the woolen textiles. No adverse effects on the rate and evenness of the dyeing have been observed, even if the treatment with the polyfunctional compound is carried out before the dyeing operation. Moreover, there is no change of shade or adverse effect on color-fastness if the treatment with the polyfunctional compound is applied to the textile after the dyeing operation. This aspect of the invention is particularly important from a commercial standpoint inasmuch as it allows a wider range of operating conditions and greater flexibility in carrying out the modification of the woolen textile product.

When carrying out the process of the invention utilizing aziridinyl compounds in combination with selected co-reactants as defined above, the treatment may be carried out in a single step or in several separate steps. Because of their nature, it is possible to use the polyfunctional compounds as defined herein in a single step in conjunction with other functional finishes such as water and stain repellents, soil release agents and the like. The latter include the acrylics and their salts as well as the fluorocarbons. The ease of formulation and application of the polyfunctional compounds makes them particularly suitable for use in combination with other finishes to impart permanent creasing properties to woolen fabrics.

No special precautions need be taken when carrying out the process of the present invention inasmuch as the insolubilization reaction of the polyfunctional compound on the wool textile can take place at moderate temperatures. It is therefore possible to obtain the desired insolubilization reaction even by tumble-drying procedures which are especially desirable when the objective is the stabilization of manufactured woven or knitted garments which cannot be conveniently processed in curing ovens at elevated temperature. Thus, the present invention provides a commercially feasible means for applying shrink-

proofing finishes to manufactured garments in a convenient or simple method without requiring the use of complex equipment and procedures.

Applicable to wool textile materials in any form or shape, the present invention may be used to impart dimensional stability and other desired properties to wool fibers, woolen and worsted yarn, woven or knitted fabrics and garments. In general, for optimum effects to be realized, the fabric customarily contains appreciable proportion of wool fiber, generally 30% or more, 60 to 100% being the preferred range.

It will be apparent from the foregoing that the wool present in the textile can be by itself or present in a blend or admixture with other natural fibers such as cotton or with synthetic fibers such as polyamides, polyesters, polyolefins and acrylic fibers. The examples which appear hereinafter generally show the reaction condition suitable for obtaining satisfactory results. It will be noted, however, that the optimum conditions for processing any given fiber blend or mixture will be determined by many factors such as concentration of reagent, time of impregnation, temperature, atmospheric conditions, configuration, as well as other parameters. Conditions within the ranges discussed hereinafter will generally give satisfactory results on the textile materials indicated although these ranges are not to be construed as limiting the invention in any way.

For most purposes, the polyfunctional compounds employed in this invention are used in amount sufficient to keep shrinkage below 6% based upon the original dimensions of the substrate. Generally between about 0.5 and 10% by weight add-on based upon the weight of the dry substrate is sufficient to keep shrinkage below the desired level. This add-on is referred to as a modifying amount of polyfunctional composition throughout this application. For example, in a typical embodiment where a 100% wool substrate is treated, add-on amounts of about 2% to about 5% based on the weight of the wool treated are preferred, although amounts outside these ranges may be used.

In accordance with the aspect of this invention relating to the combination of the aziridine compound and co-reactant, when the co-reactant is used, the amount thereof employed should be sufficient to provide approximately 0.5 to about 2.0 reactive groups of the co-reactant which is in the form of amino groups or carboxyl groups for each aziridinyl group of the aziridinyl compound defined by Formula (I). In other words, approximately 0.5 to about 2.0 equivalents of the co-reactant, polyamine or polycarboxylic acid, should be present for each aziridinyl equivalent present. It has been determined that the co-reactant may be added to the treating solution which contains the aziridinyl compound of Formula (I) or can be applied in a separate step either before or after application of the aziridinyl compound. Properties and characteristics may vary somewhat depending upon the sequence of reaction; however, it has been observed that generally the order of reactants can be varied with equally satisfactory results.

As mentioned above, the aziridinyl compound can be applied to the wool-containing textile material in any convenient manner. Generally, the aziridinyl compound is dissolved at the desired concentration in an anhydrous organic solvent such as a hydrocarbon including toluene, xylene, petroleum fractions and similar materials, halogenated solvent such as carbon tetrachloride and perchloroethylene or any other convenient inert solvent in which the aziridinyl compound is soluble and which in itself will not adversely affect the woolen textile material or deleteriously interfere with the insolubilization of the aziridinyl compound or interfere with the functioning of the co-reactant if any is used.

The aziridinyl compound may be applied to the woolen textile substrate in the form of a self-emulsifiable concentrate which is diluted with water to the desired concen-

tration prior to using same. In any event, the co-reactant polyamine or polycarboxylic acid may be added to the treating solution or emulsion containing the aziridinyl compound or the co-reactant may be applied in a separate step from a solution prepared from the same solvent as that used in connection with the aziridine compound, or a different organic solvent or water. When the co-reactant is applied in a separate step either before or after the treatment with the aziridinyl compound, the solvent from which it is deposited on the woolen textile material may be miscible or immiscible with the solvent system from which the aziridinyl compound is applied. It has been observed that the pH of the treating solution may be varied within a considerable range. Generally, very high and very low pH ranges should be avoided since degradation of the wool can occur under extreme conditions. A pH range in general of 3.0 to about 9.0 is suitable with the range of 4.0 to 8.0 being preferred for most applications.

Methods of application of the polyfunctional compounds to the woolen textile not being critical, the treating solution can be applied by any suitable means including padding, spraying, dipping or the like. Excess solution is generally removed by wringing, squeezing, centrifuging or spinning. Thereafter, the woolen textile material is dried at a temperature ranging from ambient temperature to about 100° C., the range of 50° C. to 70° C. being particularly convenient. It is to be noted that the drying step is not essential to the overall efficiency of the process. After drying, the treated textile is cured by allowing it to stand at ambient temperature for several hours or preferably by heating for a few minutes at 110° C. to about 170° C. to complete the insolubilization reaction. The time required for the curing step varies with the particular reagent and the concentrations employed. It will be noted that the curing duration will be dependent upon the temperature, the higher temperatures requiring less curing time. Curing cycles of 3 to 15 minutes at 120° C. to 150° C. have been found to give excellent results in the majority of situations. The above ranges are indicative of suitable reaction conditions and are by no means considered limiting of the present invention.

Although the textile may be used without further treatment, it is generally preferred to wash the textile after the curing step with suitable detergent solutions, solvent scours or by any other desirable means in order to remove residual soluble unreacted chemicals. The textile material can thereafter be dyed by conventional procedures or subjected to other conventional chemical or mechanical finishing operations such as shearing, topping with softeners and other textile treatments designed to impart specific properties or behavior characteristics.

The following examples are illustrative of the process of the invention. Parts are by weight unless otherwise specified. The methods used in obtaining the test data given in the examples are as follows:

Shrinkage: Measurement after laundering according to the following procedure: Samples ca. 18 x 18 inches with 10 x 10-inch markings laundered in an automatic home-type agitator washing machine at 41° C., using a 5-lb. load, detergent (Fab or Tide) and 15 minutes suds time. Washed samples were rinsed, extracted in the washer for the full cycle, dried flat on a horizontal screen and flat-bed pressed for 5 seconds at 135°-150° C. and conditioned for a minimum of 12 hours at 63 to 67% R.H. and 20-22° C. The samples were then measured for shrinkage in the warp and filling directions. Results reported in percent. The number of laundering-drying cycles is indicated by 5L or 10L, respectively.

Flex abrasion resistance: ASTM D-1175-61T (Stoll Flex Abrader, 1/2 lb. head, 2 lbs. toggle). Results reported in cycles to break.

Stiffness: Cantilever procedure. ASTM D-1388-55T. Results reported in milligram-centimeters.

Reflectance: ASTM E97-55. Photovolt 610, and Search 6104, using the green tristimulus filter.

## ABBREVIATIONS IN TABLES

When used individually:

F means filling direction, and  
W means warp direction.

OWF: On the weight of the fabric.

OWB: On the weight of the bath.

WPU: Wet pick-up.

OWB times WPU/100% = OWF.

Epoxy content—as in milliequivalents per gram: The method of aqueous magnesium chloride hydrochlorination was described in "Organic Analysis" (Interscience Publishers, Inc., New York, N.Y., 1953), vol. 1, p. 134.

Isocyanate content—as in a fraction of an equivalent per 100 grams: Determined by a modification of the dibutylamine procedure of W. Siefken, *Liebigs Annalen der Chemie*, vol. 562, p. 100 (1949).

## EXAMPLE 1

Preparation of a polyfunctional compound having (1) a backbone derived from a polyetherdiamine, and (2)



terminal 2-(1-aziridinyl)ethoxy groups

## First stage:



On the average,  $x=$ about 33 in Examples 1, 2, and 3, (and about 16 in Examples 4 and 5).



ICTID, and isocyanate-terminated intermediate having a backbone derived from a polyetherdiamine.



## Second stage:



The polyetherdiamines used as starting material had an equivalent weight of 1000 as an amine. It was marketed under the trade name Polyetherdiamine L-2000 by Union Carbide Corp. The first stage of the process consisted of converting the amine-terminated polyether into an isocyanate-terminated compound. A 1-liter jar equipped with a stirrer, a thermometer, a dropping funnel, and a vent

was charged with 200 grams of the polyetherdiamine dissolved in 200 grams of dichloromethane and cooled to  $-15\pm 5^\circ \text{ C}$ . Then, 4-methyl-*m*-phenylene diisocyanate (24.5 grams, 0.141 mole) dissolved in 50 grams of dichloromethane was added. The temperature was allowed to rise to  $25^\circ \text{ C}$ . during one hour.

Next, the second stage of adding terminal 2-(1-aziridinyl)ethoxy radicals was carried out. (1-Aziridine)ethanol (8.8 grams, 0.101 mole) was added dropwise to 19/20 of the original solution obtained from the first stage. The addition was completed in 0.5 hours, all at  $26\pm 2^\circ \text{ C}$ . The solution was stirred for 2 hours longer, after which time the infrared spectrum was devoid of the isocyanate band at 4.3 to 4.5 microns. The aziridinyl content of the product was 0.034 equivalent per 100 grams of solid (0.047 eq./100 g., calculated). The solution was miscible with dimethylformamide.

## EXAMPLE 2

20 A preparation similar to Example 1 but without substituted ethoxy as part of the terminal 1-aziridinyl-groups

For the chemical equation applying to the first stage, see Example 1,  $x=$ about 33 on the average.

## Second stage:



In the first stage, the isocyanate-terminated intermediate (ICTID) having a backbone derived from a polyetherdiamine was prepared in a manner similar to that of Example 1. The polyetherdiamine had an average equivalent weight of approximately 1000.

In the second stage, 0.127 equivalent of the isocyanate-terminated intermediate was allowed to react with 5.6 grams (0.13 mole) of ethylenimine dissolved in 50 grams of dichloromethane. The conditions were similar to those described in Example 1. The aziridinyl content was found to be 0.06 equivalent per 100 grams of solid (0.061 eq./100 g. calculated).

## EXAMPLE 3

45 A preparation similar to Example 1 but with 2,3-epoxypropyl in place of 2-(1-aziridinyl)ethoxy as the terminal groups

For the chemical equation applying to the first stage, see Example 1,  $x=$ about 33 on the average.

## Second stage:



In the first stage, the isocyanate-terminated intermediate (ICTID) having a backbone derived from a polyetherdiamine was prepared in a manner similar to that of Example 1, from the polyetherdiamine having an average equivalent weight of approximately 1000.

In the second stage, 0.109 equivalent of the isocyanate-terminated intermediate (calculated isocyanate content, 0.129 equivalent) was allowed to react with 8.06 grams (0.109 mole) of 2,3-epoxy-1-propanol. (The 2,3-epoxy-1-propanol in 50 grams of dichloromethane was added gradually over the period of an hour to the isocyanate-terminated intermediate.) After stirring for one week at room temperature, the epoxy content was found to be 0.031 equivalent per 100 grams of solid (calculated: 0.050 eq./100 g.). The infrared spectrum was devoid of the band characteristic of isocyanate at the end of the reaction period.

**13**  
**EXAMPLE 4**

A preparation similar to Example 2  
but of lower molecular weight

For the chemical equations applying, see Example 2,  
wherein  $x$ =about 16 on the average.

In the *first stage*, the isocyanate-terminated intermediate (ICTID) having a backbone derived from a polyether-diamine was prepared in a manner similar to that of Example 1. The polyetherdiamine had an average molecular weight of approximately 1000. It was marketed under

**14**

of Example 1. A 38% solution of the product in dichloromethane was diluted with dimethylformamide to give the percentages OWB shown in the accompanying table. Solutions were applied by means of a laboratory padder. After padding, the samples were framed at the original dimensions and dried at approximately 70° C. All samples were cured for 5 minutes at 135° C. The cured fabric was rinsed in dimethylformamide, then in water, again framed to the original dimensions, and dried. Very effective shrinkproofing was achieved on the wool, as the results in the accompanying table bear out.

**EXAMPLE 6**

| Sample            | Product of Example 6, percent |     |      | Actual weight gain, percent | Warp flex abrasion resistance, 0.5 x 2 lbs., cycles | Warp stiffness, mg./cm. | Green filter reflectance, percent | Shrinkage, * percent |       |      |       |
|-------------------|-------------------------------|-----|------|-----------------------------|-----------------------------------------------------|-------------------------|-----------------------------------|----------------------|-------|------|-------|
|                   | OWB                           | WPU | OWF  |                             |                                                     |                         |                                   | IL                   | 5L    | W    | F     |
| A                 | 5.0                           | 115 | 5.75 | 6.08                        | 1.250                                               | 349                     | 63                                | 1.0                  | (0.5) | 1.5  | (0.5) |
| B                 | 3.3                           | 119 | 3.93 | 5.24                        | 1.050                                               | 334                     | 63                                | 2.0                  | (0.5) | 2.5  | (1.0) |
| C                 | 1.7                           | 124 | 2.11 | 3.85                        | 1.050                                               | 262                     | 63                                | 2.5                  | (0.5) | 4.0  | (1.5) |
| D                 | 0.8                           | 121 | 0.97 | 3.19                        | 850                                                 | 203                     | 62                                | 3.5                  | (0.5) | 5.5  | (1.0) |
| Untreated control |                               |     |      |                             | 725                                                 | 127                     | 62                                | 15.0                 | 3.5   | 27.5 | 15.0  |

\*Percentages in parentheses are the opposite of shrinkage.

the trade name Polyetherdiamine L-1000 by Union Carbide Corp.

In the *second stage*, 0.223 equivalent of the isocyanate-terminated intermediate was allowed to react with 10.5 grams (0.244 mole) of ethylenimine dissolved in 50 grams of dichloromethane. Conditions were similar to those described in Example 1. The aziridinyl content was found to be 0.11 equivalent per 100 grams of solid (0.13 eq./100 g., calculated). The infrared spectrum of the product was devoid of the isocyanate band.

**EXAMPLE 5**

A preparation similar to Example 1  
but of lower molecular weight

For the chemical equations applying, see Example 1,  
wherein  $x$ =about 16 on the average.

The procedure for the *first stage* was similar to that stated in Example 4.

In the *second stage*, 0.166 equivalent of the isocyanate-terminated intermediate was allowed to react with 0.166

**EXAMPLE 7**

Dimensional stabilization using the product of Example 2

Samples of the 100% woolen fabric weighing 6.15 oz./sq. yd. were treated according to the general procedure of Example 6 with the following variations: The reagent was the product of Example 2. A 40% solution of it in dichloromethane was diluted with dimethylformamide to give the percentages OWB shown in the accompanying table. For the preparation of the "E" and "F" series of samples, the pad bath also contained tetraethylenepentamine (TEPA). The concentration of TEPA was approximately 9% of the concentration of the product of Example 2 OWB. After padding, samples were dried at approximately 65° C. Quantitative details and curing conditions are in the accompanying table, as are the evaluation results of the use of the reactive polymer having a backbone made up of repeating propyleneoxy units and having terminal amide-type 1-aziridinyl groups.

TABLE TO EXAMPLE 7

| Wool fabric sample | Product of Example 2, percent |     |     | TEPA, OWF, percent | Cure, 5 min. at ° C. | Actual weight gain, percent | Warp flex abrasion resistance, 0.5 x 2 lbs., cycles | Warp stiffness, mg./cm. | Shrinkage, * percent |       |      |      |
|--------------------|-------------------------------|-----|-----|--------------------|----------------------|-----------------------------|-----------------------------------------------------|-------------------------|----------------------|-------|------|------|
|                    | OWB                           | WPU | OWF |                    |                      |                             |                                                     |                         | IL                   | 5L    | W    | F    |
| A1                 | 5.2                           | 123 | 6.4 | None               | 135                  | 1.6                         | 800                                                 | 140                     | 9.0                  | (1.5) | 13.5 | 3.0  |
| A2                 | 5.2                           | 129 | 6.7 | None               | 163                  | 3.0                         | 825                                                 | 220                     | 2.0                  | None  | 3.0  | 0.5  |
| B1                 | 3.4                           | 125 | 4.2 | None               | 135                  | 1.8                         | 950                                                 | 140                     | 7.0                  | None  | 11.5 | 3.0  |
| B2                 | 3.4                           | 118 | 4.1 | None               | 163                  | 1.5                         | 900                                                 | 128                     | 7.0                  | 0.5   | 11.0 | 3.5  |
| E1                 | 5.2                           | 132 | 6.8 | 0.6                | 135                  | 3.2                         | 975                                                 | 178                     | 5.5                  | None  | 7.0  | None |
| E2                 | 5.2                           | 122 | 6.3 | 0.6                | 163                  | 3.5                         | 1,000                                               | 198                     | 4.5                  | (0.5) | 6.5  | None |
| F1                 | 3.4                           | 123 | 4.2 | 0.4                | 135                  | 2.8                         | 1,000                                               | 128                     | 5.0                  | (1.0) | 8.0  | None |
| F2                 | 3.4                           | 119 | 4.1 | 0.4                | 163                  | 2.5                         | 750                                                 | 120                     | 7.0                  | 0.5   | 8.0  | 0.5  |
| Control untreated  |                               |     |     |                    |                      |                             | 725                                                 | 114                     | 15.0                 | 3.5   | 27.5 | 15.0 |

\*Percentages in parentheses are the opposite of shrinkage.

mole of (1-aziridine)ethanol in a manner similar to that used in Example 1. The aziridinyl content of the product was 0.09 equivalent per 100 grams of solid (0.10 eq./100 g., calculated). The infrared spectrum of the product was devoid of the isocyanate band. The product was very soluble in dimethylformamide.

**EXAMPLE 6**

Dimensional stabilization of woolen fabric by treatment with the product of Example 1

Samples of the 100% woolen fabric weighing 6.15 oz./sq. yd. were treated according to quantitative details in the accompanying table with solutions of the product

**EXAMPLE 8**

Dimensional stabilization using the product of Example 3

A procedure similar to that of Example 7 was followed, using the product of Example 3, a polymer whose central moiety had repeating propyleneoxy groups, and whose terminal groups were 2,3-epoxypropoxy groups. A 42% solution of the product in dichloromethane was diluted with dimethylformamide to give the percentages OWB shown in the accompanying table. All samples were cured for 5 minutes at 135° C. As is evident from the evaluation results, improved dimensional stabilization re-

sulted from the use of the product of Example 3, especially when tetraethylenepentamine also was used.

TABLE TO EXAMPLE 8

| Wool fabric sample | Product of Example 3, percent |     |     | Actual weight gain, percent | Warp flex abrasion resistance 0.5 x 2 lbs., cycles | Shrinkage, percent      |      |             |      |
|--------------------|-------------------------------|-----|-----|-----------------------------|----------------------------------------------------|-------------------------|------|-------------|------|
|                    | OWB                           | WPU | OWF |                             |                                                    | Warp stiffness, mg. cm. | 1L W | 1L F        | 5L W |
| B                  | 3.6                           | 125 | 4.5 | None                        | 2.9                                                | 1,050                   | 145  | 6.5         | None |
| C                  | 2.7                           | 124 | 3.3 | None                        | 2.5                                                | 1,025                   | 146  | 8.0         | None |
| E                  | 0.9                           | 121 | 1.1 | None                        | 2.5                                                | 870                     | 171  | 6.5         | None |
| G                  | 3.6                           | 129 | 4.6 | 0.9                         | 5.7                                                | 1,050                   | 587  | 2.0         | None |
| H                  | 2.7                           | 125 | 3.4 | 0.6                         | 4.1                                                | 1,015                   | 449  | 1.5 * (0.5) | 3.0  |
| J                  | 0.9                           | 129 | 1.1 | 0.2                         | 2.8                                                | 1,025                   | 308  | 2.0         | None |
| Control untreated  |                               |     |     |                             |                                                    | 725                     | 114  | 15.0        | 3.5  |
|                    |                               |     |     |                             |                                                    |                         |      |             | 27.5 |
|                    |                               |     |     |                             |                                                    |                         |      |             | 15.0 |

\*The opposite of shrinkage.

## EXAMPLE 9

## Dimensional stabilization using the product of Example 4

A procedure similar to that of Example 8 was followed, using the product of Example 4, a polymer whose central moiety had repeating ethyleneoxy groups (fewer than the product of Example 2), and whose terminal groups were amide-type 1-aziridinyl groups. A 41% solution of the product in dichloromethane was diluted with dimethylformamide to give the percentages OWB shown in the accompanying table. All samples were cured for 5 minutes at 135° C. Excellent dimensional stabilization was obtained, whether in the presence of tetraethylenepentamine or without it.

TABLE TO EXAMPLE 9

| Wool fabric sample | Product of Example 4, percent |     |     | Actual weight gain, percent | Warp flex abrasion resistance 0.5 x 2 lbs., cycles | Shrinkage, percent      |      |      |      |
|--------------------|-------------------------------|-----|-----|-----------------------------|----------------------------------------------------|-------------------------|------|------|------|
|                    | OWB                           | WPU | OWF |                             |                                                    | Warp stiffness, mg. cm. | 1L W | 1L F | 5L W |
| A                  | 5.2                           | 123 | 6.4 | None                        | 5.5                                                | 1,325                   | 711  | 0.1  | 1.0  |
| B                  | 3.4                           | 127 | 4.3 | None                        | 3.2                                                | 1,050                   | 398  | 1.5  | 1.0  |
| D                  | 0.85                          | 129 | 1.1 | None                        | 2.5                                                | 1,250                   | 602  | 2.5  | None |
| E                  | 5.2                           | 125 | 6.5 | 1.3                         | 4.8                                                | 1,200                   | 610  | 1.5  | None |
| F                  | 3.4                           | 125 | 4.2 | 0.8                         | 6.7                                                | 1,550                   | 475  | 0.5  | None |
| H                  | 0.85                          | 128 | 1.1 | 0.3                         | 4.5                                                | 700                     | 599  | 3.0  | 0.5  |
| Control untreated  |                               |     |     |                             |                                                    | 725                     | 114  | 15.0 | 3.5  |
|                    |                               |     |     |                             |                                                    |                         |      |      | 27.5 |
|                    |                               |     |     |                             |                                                    |                         |      |      | 15.0 |

## EXAMPLE 10

## Dimensional stabilization using the product of Example 5

A procedure similar to that of Example 9 was followed, using the product of Example 5, a polymer whose central moiety had repeating propyleneoxy groups (fewer than the product of Example 1), and whose terminal groups were 2-(1-aziridinyl)ethoxy groups. A 20% solution of the product in dichloromethane was diluted with dimethylformamide to give the percentages OWB shown in the accompanying table. All samples were cured for 5 minutes at 135° C. Evaluation results in the accompanying table indicate that the reactive derivative of a polyetherdiamine is a very effective shrinkproofing agent.

TABLE TO EXAMPLE 10

| Wool fabric sample | Product of Example 5, percent |     |     | Actual weight gain, percent | Warp flex abrasion resistance 0.5 x 2 lbs., cycles | Shrinkage, percent      |      |      |      |
|--------------------|-------------------------------|-----|-----|-----------------------------|----------------------------------------------------|-------------------------|------|------|------|
|                    | OWB                           | WPU | OWF |                             |                                                    | Warp stiffness, mg. cm. | 1L W | 1L F | 5L W |
| A                  | 5.2                           | 126 | 6.6 | 7.8                         | 1,375                                              | 715                     | 0.5  | 0.5  | 1.0  |
| B                  | 3.4                           | 127 | 4.3 | 6.9                         | 1,125                                              | 706                     | 0.5  | 0.5  | 1.0  |
| C                  | 1.7                           | 133 | 2.2 | 5.8                         | 975                                                | 483                     | 1.5  | None | 3.0  |
| D                  | 0.85                          | 130 | 1.1 | 4.5                         | 700                                                | 253                     | 3.5  | None | 5.5  |
| Control untreated  |                               |     |     |                             | 725                                                | 114                     | 15.0 | 3.5  | 27.5 |
|                    |                               |     |     |                             |                                                    |                         |      |      | 15.0 |

It is understood that various other modifications will be apparent to and can readily be made by those skilled in the art without departing from the scope and spirit of this invention. Accordingly, it is not intended that the scope of the claims appended hereto be limited to the description set forth herein but rather that the claims be construed as encompassing all the features of patentable novelty which reside in the present invention, including

all features which would be treated as equivalents thereof by those skilled in the art to which the invention pertains.

## 16

## What is claimed is:

1. A process for improving the dimensional stability of wool-containing fabrics comprising applying to said fabric a polyfunctional compound of the formula



wherein

A is an epoxyalkoxy group;

m is an integer from 2 to 3;

R is hydrogen or alkyl of from 1 to 5 carbon atoms;

J is a member selected from the group consisting of

$(-\text{CH}_2-)_x$ , where x is an integer from 1 to 100;

$(-\text{C}_a\text{H}_{2a}\text{O})_x\text{C}_a\text{H}_{2a}$ , where a is an integer of

from 1 to 4 and x has the meaning given above;

$(-\text{CH}_2\text{CH}=\text{CHCH}_2-)_u$ , where u is an integer of from 6 to 100;



where

a and x have the meanings given above;

y is an integer of from 1 to 100; and

L is alkylene of 2 to 20 carbon atoms or alkylene of 2 to 20 carbon atoms having the chain interrupted by 1 to 10



where R is alkyl of 1 to 5 carbon atoms; and



and Q is a member selected from the group consisting of phenylene, methylphenylene, phenylenedimethylene, biphenylene, methylenediphenylene, benzylphenylene and naphthylene,

said polyfunctional compound being applied from a liquid medium, and insolubilizing said polyfunctional compound on said fabric.

2. A process as claimed in Claim 1 wherein said polyfunctional compound is applied to said fabric in the form of a solution in an anhydrous solvent.

3. A process as claimed in Claim 1 wherein said polyfunctional compound is applied to said fabric in the form of an aqueous solution.

4. A process as claimed in Claim 1 wherein said polyfunctional compound is applied to said fabric in the form of an aqueous emulsion.

5. A process as claimed in Claim 1 wherein A is an epoxypropoxy group of the formula



6. A process as claimed in Claim 1 wherein said polyfunctional compound is insolubilized by curing at a temperature of about 100° C. to 200° C.

7. A process as claimed in Claim 1 where in addition to said polyfunctional compound there is applied to said fabric a polyalkylene polyamine and said polyalkylene polyamine is coreacted with said polyfunctional compound during said insolubilization.

#### References Cited

#### UNITED STATES PATENTS

|    |           |         |         |       |           |
|----|-----------|---------|---------|-------|-----------|
| 10 | 2,327,760 | 8/1943  | Bestian | ----- | 8—Oxirane |
|    | 3,165,375 | 1/1965  | Tesoro  | ----- | 8—127.6   |
|    | 3,248,280 | 4/1966  | Hyland  | ----- | 8—Oxirane |
|    | 3,279,882 | 10/1966 | Tesoro  | ----- | 8—127.6   |

15 LEON D. ROSDOL, Primary Examiner

H. WOLMAN, Assistant Examiner

U.S. Cl. X.R.

20 8—115.7, 128 R, 128 A, Digest 8; 260—348

UNITED STATES PATENT OFFICE  
CERTIFICATE OF CORRECTIONPatent No. 3,832,132Dated August 27, 1974Inventor(s) Giuliana C.Tesoro, Stephen B.Sello and Rudolf F.Wurster

It is certified that error appears in the above-identified patent and that said Letters Patent are hereby corrected as shown below:

Column 4, line 39, should read -- L is a divalent alicyclic radical of 3 to 20 carbon --. Column 5, under "Starting Compounds, etc." (the 7th compound) 1,4-cyclohexanedimethanol - in the formula should read



Column 5, formula at the bottom of the page, at the right side should read



Column 8, line 55, "tied" should read -- ried --. Column 11, line 66, Second stage Formula, last ring, should read



Columns 13 and 14, Example 6 Table, under "Green filter reflectance percent" the sample "Control untreated" "62" should read -- 65 --.

Signed and sealed this 15th day of April 1975.

(S.E.M.)

Attest:

RUTH C. MASON  
Attesting OfficerC. MARSHALL DANN  
Commissioner of Patents  
and Trademarks